

## UNITED STATES PATENT OFFICE

2,153,973

## LUBRICATING OILS

Raphael Rosen, Cranford, and Robert M. Thomas,  
Elizabeth, N. J., assignors to Standard Oil De-  
velopment Company, a corporation of Delaware

No Drawing. Application November 10, 1933,  
Serial No. 697,470

2 Claims. (Cl. 87—9)

The present invention relates to improved lub-  
bricating oils and methods for producing them,  
and particularly to oils of low oxidation rate and  
low sludging tendency. The invention will be  
fully understood from the following description:

It has long been observed that well refined oils  
show a higher rate of oxidation than the un-  
refined oils from which they are obtained. This  
has been attributed to the fact that refining  
methods remove certain materials which inhibit  
oxidation and this apprehension seems to be  
plausible because inhibiting substances are known  
which can be added to oils to greatly reduce their  
oxidation rates. Among the known inhibitors  
are phenolic substances such as the cresols, naph-  
thols and anthrols. For some purposes these  
materials serve excellently. However, it has been  
found that the addition of these materials always  
tends to increase the sludging tendency of the oil,  
for example, as measured by the Sligh test, see  
Proceedings of the American Society for Testing  
Materials, 24, 984, II (1924).

A new class of inhibitors has now been discovered  
which are not only much more powerful  
than the phenolic inhibitors, but which actually  
reduce the sludging tendency of the oils. These  
materials comprise certain sulfur compounds  
specifically aliphatic and aromatic polysulphides  
and the corresponding polyselenides and poly-  
tellurides. By the term "polysulfide" we intend  
to include only substances of the following gen-  
eral formula



35 This does not include, however, the well known  
disulphides of the general formula



40 In each of the above formulae the  $R+R'$  denotes  
alkyl or aryl groups. The  $x$  may represent 1 or  
more sulphur atoms. This is preferably under 3  
since the penta and higher sulphides are corro-  
sive while those below 3 are not.

The present inhibitors can be used in any type  
of well refined hydrocarbon oils from the light  
spindle to the heaviest lubricating oils. They  
are most desirable, however, when used in oils of  
50 a strongly paraffinic nature such as those derived  
from paraffin base crudes, or from oils which  
have been extracted with agents of the type of  
phenol, cresol, sulfur dioxide, nitrobenzol and  
dichlorethyl ether, all of which have the property  
55 of removing the non-paraffinic constituents.  
These inhibitors are also well suited to oils pre-  
pared by hydrogenation or destructive hydrogen-  
ation, and to oils refined by vigorous action with  
concentrated and even fuming sulfuric acid; in  
60

other words, the so-called white mineral oils.  
They are likewise useful in waxes and in the syn-  
thetic oils prepared by chemical or electrical con-  
densation.

While essentially paraffinic oils described above  
are the most important ones, it is worth noting  
that the present inhibitors are also effective in  
reducing the oxidation rate of naphthenic or as-  
phaltic oils which have been well refined. This  
is a most unusual and unexpected property and  
may be taken as an indication that these inhibi-  
tors are different in their action from those for-  
merly used, namely, the phenolic, because these  
latter show no appreciable reduction of the oxida-  
tion rate of naphthenic oils, whereas, the pres-  
ent agents show a very substantial reduction.

The present inhibitors may be used in rela-  
tively small amounts, say as low as .01% for  
highly refined oils such as "white" oils or less re-  
fined oils in the lower range of temperatures, say 20  
below 150° C. but usually they are preferred in  
somewhat larger amounts for example, .05 to  
0.1% and as much as 1% can be used at higher  
temperatures although this is not necessary and  
is usually undesirable. They may be added di-  
rectly to the finished lubricating oil in any de-  
sired form for example, directly or in a suitable  
solvent, such as carbon disulfide or carbon teta-  
chloride or the like, and then incorporated with  
the oil. The solvent may be removed by distilla-  
tion with steam, or under vacuum.

35 It is preferred to add pure agents but oils known  
to contain these materials may be added to the  
refined oils so as to incorporate the desired quan-  
tities of the inhibitors. It should also be under-  
stood that the sulfur compounds should be added  
after all of the refining steps have been com-  
pleted because the usual refining methods will  
remove sulfur compounds and their equivalent.  
It will be understood, of course, that if the type  
40 of refinement is such as not to accomplish the  
removal of sulfur, then the agents may be added  
prior to such treatment.

45 Most of the above mentioned substances are of  
the type known as corrosive in that they tarnish  
copper and brass but it has been determined that  
this is of little consequence, especially where  
engines are run at elevated temperatures, for ex-  
ample aeroplane engines, but some of the sub-  
stances are not corrosive. These latter are, there-  
fore, preferable. They can be made by reaction  
50 of unsaturated hydrocarbons and sulfur or sulfur  
chloride or the corresponding selenium and tellu-  
rium compounds. Cracked oils, for example,  
cracked wax may be used to produce good non-  
corrosive substances, or fatty acid containing un-  
saturated group such as lard oil. Another  
method of producing polysulfide is by treatment  
55 of a mercaptan with sodium plumbite adding  
enough sulphur to make the desired polysulfide.

The following examples are given to illustrate the use of the present inhibitors and the properties of the inhibited oils:

*Example I*

- 5 The blank oil base used in this test was a well refined lubricating oil having a Saybolt viscosity of 145 seconds at 100° F. The inhibitor consisted of butyl pentasulphid prepared by treating butyl mercaptan with sodium plumbite and sulfur, sufficient to form the polysulphid indicated. The oxidation was conducted on a 10 cc. sample, agitating with a definite quantity of oxygen at 200° C. The absorption of oxygen was measured in cubic centimeters at 15 minute intervals.

| Time intervals | Blank | Blank +0.1% butyl pentasulphid |
|----------------|-------|--------------------------------|
| 1              | 160   | 8                              |
| 2              | 135   | 8                              |
| 3              | 65    | 72                             |
| 4              | 42    | -----                          |

- 10 15 This material was corrosive and did not exert its effect as long as might be desired.

*Example II*

- 10 The blank used in this experiment was a well refined motor oil S. A. E. Grade 50. The polysulphid inhibitor was produced by reacting wax fractions (boiling 200 to 600° F.) at 150 to 200° C. with 10% S<sub>2</sub>Cl<sub>2</sub>. The product contained 2½% sulfur and a small amount of chlorine which was removed by treatment with alcoholic soda. The tests were conducted as in the prior example.

| Time intervals | Blank | 1% polysulphid inhibitor |
|----------------|-------|--------------------------|
| 1              | 132   | 22                       |
| 2              | 116   | 20                       |
| 3              | 32    | 22                       |
| 4              | 49    | 20                       |

*Example III*

To the same blank as used in Example II an inhibitor is added prepared by cooking lard oil at 150 to 200° C. with, approximately, 10% sulfur. The tests were conducted as before.

| Time interval | Blank | 0.1% inhibitor | 0.25% inhibitor |
|---------------|-------|----------------|-----------------|
| 1             | 132   | 32             | 15              |
| 2             | 116   | 47             | 20              |
| 3             | 32    | 56             | 21              |
| 4             | 49    | -----          | 21              |

5

10

15

20

25

With the present inhibitor .1% is too small to be effective for the entire test at the high temperature used but its influence is clearly perceptible. At lower temperatures this amount is sufficient but at 200° C. it is preferable to use .25% which is altogether satisfactory.

The present invention is not to be limited by any theory of inhibitor action nor to any particular inhibitors nor to any particular oils containing them, but only to the following claims in which it is desired to claim all novelty inherent in the invention.

We claim:

1. An improved oil composition resistant to deterioration at elevated temperatures of the order encountered in an internal combustion engine comprising a viscous hydrocarbon lubricating oil and less than 1% of an organic polysulfide prepared by reaction of a mercaptan with sodium plumbite and sulfur, the latter being sufficient to produce a polysulfide containing more than two sulfur atoms to the molecule.

2. An improved lubricating composition resistant to deterioration at elevated temperatures of the order encountered in an internal combustion engine comprising a viscous hydrocarbon lubricating oil and less than 2% of butyl pentasulfide.

RAPHAEL ROSEN,  
ROBERT M. THOMAS.

45